

(No Model.)

E. SAMUEL.

PROCESS OF MAKING COMPOSITE ARTICLES OF MANGANESE STEEL  
AND CAST METAL.

No. 599,636.

Patented Feb. 22, 1898.



Witnesses

Hamilton D. Turner  
Will. A. Raw.

Inventor:

Edward Samuel  
by his Attorneys  
Norcom & Norcom

# UNITED STATES PATENT OFFICE.

EDWARD SAMUEL, OF PHILADELPHIA, PENNSYLVANIA, ASSIGNOR TO THE  
WILLIAM WHARTON, JR., & COMPANY, INCORPORATED, OF SAME PLACE.

## PROCESS OF MAKING COMPOSITE ARTICLES OF MANGANESE STEEL AND CAST METAL.

SPECIFICATION forming part of Letters Patent No. 599,636, dated February 22, 1898.

Application filed November 3, 1894. Serial No. 527,808. (No specimens.)

*To all whom it may concern:*

Be it known that I, EDWARD SAMUEL, a citizen of the United States, residing in Philadelphia, Pennsylvania, have invented certain 5 Improvements in the Process of Hardening and Toughening Objects of Manganese Steel, of which the following is a specification.

The object of my invention is to increase the hardness and toughness of manganese- 10 steel castings, an object which I attain in the manner hereinafter set forth, reference being had to the accompanying drawing, which represents in section the preferred method of carrying my invention into effect.

15 I have found by experiment that ordinary manganese-steel castings which have been hardened by "quenching"—that is to say, by dipping them in water while highly heated—may be greatly improved both in hardness 20 and in toughness by reheating and gradually cooling the same in a certain manner. While such reheating and gradual cooling may be accomplished in any proper way, an effective and economical method of accomplishing it is 25 by casting molten iron or other molten metal in contact with the manganese-steel casting,

for in this way not only is said casting properly heated, but it can at the same time be united in a composite structure of which the 30 cast metal forms a part. For instance, in the drawing, *a* represents a manganese-steel casting, and *b* a mass of cast-iron which has been poured into contact with said steel casting

and which is firmly united thereto. The casting may be effected in any suitable mold, such 35 as that shown in section, the letter *A* indicating the cope, and *B* the drag, with the parting-line at *C*. By this means the manganese-steel castings can be used in such parts of composite structures as are subjected to the greatest 40 wear, the quality of additional hardness and toughness imparted by this treatment being of especial value in such cases.

Having thus described my invention, I claim and desire to secure by Letters Patent—

The process herein described of making a composite structure of manganese steel and cast metal, whereby the manganese steel is hardened and toughened, said process consisting in making a cast shape of manganese steel, hardening the said cast shape, then placing it in a mold, and casting molten metal in contact with it, whereby the said shape is reheated, then gradually cooling the composite structure thus formed, to harden and toughen the manganese-steel shape, substantially as described.

In testimony whereof I have signed my name to this specification in the presence of two subscribing witnesses.

EDWARD SAMUEL.

Witnesses:

WILL. A. BARR,  
JOSEPH H. KLEIN.